

## UNITED STATES PATENT OFFICE.

ADOLPHE JOUVE AND ANDRÉ HELBRONNER, OF PARIS, FRANCE

## PROCESS FOR THE MANUFACTURE OF CHROMATES AND BICHROMATES.

No Drawing.

Application filed March 14, 1922. Serial No. 543,769.

*To all whom it may concern:*

Be it known that we, ADOLPHE JOUVE and ANDRÉ HELBRONNER, citizens of the Republic of France, residing at Paris, Department 5 of the Seine, in France, and having P. O. addresses, the first 1 Boulevard Saint-Germain and the second 79 Boulevard Malesherbes, in the said city, have invented certain new and useful Improvements in a 10 Process for the Manufacture of Chromates and Bichromates; and we do hereby declare the following to be a full, clear, and exact description of the invention, such as will enable others skilled in the art to which it 15 appertains to make and use the same.

This invention has for its object improvements in processes for obtaining alkali chromates and bichromates electrolytically.

The electrolytic manufacture of alkali 20 chromates has hitherto given rise to serious errors owing to the method used, this being the electrolysis of metallic chromium or of a chromium alloy with an electrolyte formed of the alkali salt of a fixed acid.

25 These processes tend to produce chromic acid, setting free at the same time the fixed acids of the alkali salts and these different acids would require subsequently, in the course of the manufacture, to be neutralized 30 by a hydroxide composition added from time to time. In like manner and during the operation, the metal alloyed with the chromium is precipitated by this addition of hydroxide.

35 The process which forms the subject matter of the present invention consists in electrolyzing directly a chromium alloy (such as the ferrochromiums) in an electrolyte of alkali carbonate, such as sodium carbonate.

40 As a result of the reactions, the chromic acid which is formed is immediately converted into a stable alkali chromate. Furthermore there can be no free acidity arising from the fixed acids.

45 The acidity due to  $\text{CO}_2$  disappears immediately, this compound being evolved in part in the free state while the other part is saturated by the oxide of iron which is produced during the electrolysis of the ferrochromium.

The addition of hydroxide in the present process is therefore unnecessary. In reality the neutralization and the precipitation of the oxide of iron are effected by virtue of 55 the nature of the electrolyte which, during the whole of the operation, remains con-

stantly alkaline and never presents any trace of acidity. The electrolysis is carried out without the use of diaphragms. Besides the electrical resistance of the diaphragm 60 which is thus dispensed with, there is also avoided the very rapid warping which would be due to the oxide of iron penetrating into the pores of the said diaphragm, thus rendering ineffective all cleaning, however frequently it may be done, and soon rendering the apparatus useless. Finally there can no longer be any formation of chromates of aluminium and lime by the decomposition of the material of which the diaphragm is composed, viz, silicate of alumina and lime. 70

As a result of the instant invention, the electrolyzation is continuous and production of the chromates proceeds uninterruptedly, until either the electrolyte or the electrode 75 containing the chromium is exhausted, with a constant increase in the concentration of the chromate.

It also permits:

1. Of effecting the electrolysis in a constantly alkaline medium. 80

2. Of avoiding an addition of alkaline hydroxide or of lime during the electrolysis.

3. Of obtaining the automatic and constant precipitation of the iron, in the form of oxide or carbonate, eliminating this product in proportion. 85

4. Of preventing the adhesion of ferric deposits, both by the fact of the temperature of the electrolyte and by the evolution of the carbonic acid produced. 90

5. Of avoiding the separation subsequently of any deposit, such as sulphate of lime, which would be produced by the saturation of the acidity fixed by the lime in the other processes. 95

Experience has shewn that when all the carbonate has disappeared in consequence of its transformation into chromate, the electrolysis nevertheless continues to go on regularly. This is because the chromate then acts as an electrolyte exactly as the carbonate did previously. A second molecule of chromium thus becomes dissolved and the neutral chromate is converted progressively into bichromate up to the integral transformation into bichromate. 100

It has been found that in the production of bichromates, the concentration in bichromate formed has no action on the progress of the electrolysis, and therefore on the for- 110

mation of this salt. It is thus even possible, if necessary, to arrive at a concentration of such strength that the liquid crystallizes by being cooled down. For example solutions containing from 70 to 80 per cent of bichromate can be obtained without any variation of the electrolytic efficiency in the course of the operation, all other things being equal.

On the other hand, if it be desired to obtain chromate and not bichromate, the electrolysis will be pushed forward until bichromate is formed and neutral chromate then reverted to, by direct saturation of the concentrated solution of bichromate by a neutral alkali carbonate.

It is unnecessary in this case to trouble about the quantity of carbonate to be added, as it has been seen that an excess of carbonate will not dissolve in very concentrated solutions of alkali chromate.

The above explanation shows that it is possible to install a process of manufacture of alkali bichromates, in a direct manner and in a single operation by anodic electrolysis of ferrochromium in an alkaline electrolyte, preferably, in concentrated solutions of carbonate. The concentration may be effected during the electrolysis itself, by re-adding carbonate until the liquid, after its transformation into bichromate, becomes of a concentration near that at which it crystallizes by cooling down. In practice it is not necessary, however, to push this concentration as far as crystallization in order to be able to first separate the oxide of iron, by filtration for example; a slight concentration is then sufficient by application of heat in order to obtain crystallization or even solidification.

The products obtained, i. e. bichromates and subsidiarily neutral chromates, are rigorously exempt from iron and such alkali salts as carbonates.

The installation for carrying out the process, comprises substantially a series of electrolyzing tanks containing alternate series of anodes of cast ferrochromium and cathodes of lead for example. The liquid circulates from one tank to the other, in which it is subjected to the action of the current. In view of the large number of amperes (several hundred amperes per square metre) which it is possible to use, the electrolyte heats up rapidly, the operation therefore taking place in the presence of heat.

As a practical example of the application of the method, an electrolytic cell was employed, with two anodes, each approximately 30 cm  $\times$  62 cm  $\times$  5 cm consisting of 80% Cr, 33.1% Fe and 5.2% Si and C, with two lead cathodes of corresponding size, immersed in a bath of 304 liters of sodium carbonate solution containing 169.3 gr. per liter.

The electrolyzation was carried out in

twelve stages or periods, as indicated in the following table, which indicates the time intervals and the average amperage and voltage of the current employed during each period:

70

|         | Number of hours. | Mean amperage. | Mean voltage. |    |
|---------|------------------|----------------|---------------|----|
| 1.....  | 38               | 800            | 7.27          | 75 |
| 2.....  | 20 <sup>1</sup>  | 729            | 6.6           |    |
| 3.....  | 19 <sup>1</sup>  | 800            | 6.35          |    |
| 4.....  | 23 <sup>1</sup>  | 800            | 6.14          |    |
| 5.....  | 22 <sup>1</sup>  | 786            | 5.60          |    |
| 6.....  | 22 <sup>1</sup>  | 785            | 5.27          |    |
| 7.....  | 18 <sup>1</sup>  | 1. 140         | 7.27          |    |
| 8.....  | 2 <sup>1</sup>   | 1. 443         | 10.20         |    |
| 9.....  | 14 <sup>1</sup>  | 804            | 6.30          | 80 |
| 10..... | 20 <sup>1</sup>  | 1. 015         | 6.57          |    |
| 11..... | 22 <sup>1</sup>  | 1. 116         | 8.00          |    |
| 12..... | 3                | 700            | 13.75         |    |

During period 1 to 4 inclusive, sodium chromate was formed and from periods 5 to 7 the chromate was changed to bi-chromate. At this stage the operation was stopped in order to filter the liquid, and 30 liters of the filtrate was taken for the purpose of extracting the crystals by evaporation. From stages 7 to 12 bichromate of sodium was continuously obtained by electrolyzation of the residual filtrate which had been returned to the apparatus, solid carbonate of soda being added regularly during the seventh stage, but the quantity of the addition being not sufficient to effect the production of the chromate. When the operation was suspended at the end of the twelfth stage, the cell contained approximately 140 liters of mud, the liquid proportion of which contained 577 grams per liter of sodium bi-chromate with 2 molecules of water, which was readily crystallized by cooling.

Large quantities of oxide of iron are formed and although this has no influence of itself on the electrolysis, it is well to avoid too great an accumulation thereof. The oxide of iron will therefore be separated from time to time in the course of the operation, either by agitating and then filtering the liquid which is returned to the tanks, or it may be removed by centrifugal action.

Instead of using anodes of ferrochromium fused in the electric furnace, chromite may be mixed with carbon and an agglomerant such as pitch and the briquettes thus obtained submitted to a temperature sufficient to produce the total, or at least the partial reduction of the oxide of chromium, this reduction being effected by fire, without reaching the point of fusion, and furnishing a conglomerate which will be suitable for use as anodes.

Finally, experience has also shown that the preceding electrolysis may be carried out by alternating currents instead of continuous currents, provided that the density of the amperage used for the reaction be extremely high. In this way all the advan-

85

90

95

100

105

110

115

120

125

130

tages of the alternating current may be profited by.

Claims:

1. The method of producing a chromium salt of an alkali which comprises electrolyzing a solution of an alkali carbonate with an anode containing substantial proportions of chromium.
2. The method of producing chromates of alkali metals which comprises electrolyzing a solution of the carbonate of the desired alkali metal with an anode containing chromium in substantial proportions.

3. The method of producing chromates and bichromates of alkali metals which comprises electrolyzing a solution of the carbonate with an anode containing substantial proportions of chromium to first form alkali chromate, and continuing the electrolytic action to convert the resultant chromate into bichromate.

In testimony whereof we affix our signature.

ADOLPHE JOUVE.

ANDRÉ HELBRONNER.